

## UNITED STATES PATENT OFFICE

2,142,024

## COATING SURFACES OF ZINC-BASE

William E. Hall, Hillside, N. J., assignor to The  
Egyptian Lacquer Manufacturing CompanyNo Drawing. Application September 30, 1936,  
Serial No. 103,362

7 Claims. (Cl. 91—68)

This invention relates to coating metallic surfaces, especially surfaces of inherently water-repellant metals, for example, zinc, cadmium, or magnesium or alloys of these elements in which 5 zinc or cadmium or magnesium or two or three of these elements constitute a major ingredient. The invention is adapted for coating galvanized surfaces and the like and contemplates particularly the production of decorative and protective 10 coatings on sheet metal products such as galvanized iron roofing or shingles.

Galvanized iron surfaces tend to tarnish and corrode upon exposure to the weather and leave 15 much to be desired from the standpoints of appearance and durability unless subjected to further treatment. Consequently it has been heretofore customary practice to paint the galvanized metal either before or after it is in place. Paint tends to peel after a short time of service 20 when applied to untreated galvanized surfaces so that it has been proposed heretofore to etch or sandblast the galvanized surfaces preparatory to applying the paint. Etching, however, has not proved entirely satisfactory because zinc, and 25 particularly zinc in crystalline form on galvanized surfaces, tends to etch in an irregular and spotty manner which deleteriously affects both the appearance and the resistance to weather of the finished surface.

Spray application of primer and paint to galvanized metal, especially galvanized metal roofing which is coated at the factory in large lots, is 30 highly desirable because of the resultant saving in labor. But efforts to employ the heretofore customary etching agents or "primers", such as aqueous solutions of hydrochloric acid, to the galvanized metal by means of sprays has only aggravated the aforementioned difficulties. When 35 applied with sprays such primers do not flow uniformly over the galvanized roofing but tend to collect as isolated droplets. Etching occurs immediately adjacent the droplets but, unless an excessive amount of primer is sprayed on, much of the surface area remains unetched while other 40 portions are excessively corroded. When the surface is etched in this uneven manner, the lack of uniformity in appearance persists even after the surface is painted, probably because the more deeply etched surfaces absorb more of the paint 45 vehicles than other portions and form spots which have less lustre than adjacent areas. Such spots of lower lustre are similar in appearance to those known as "hot spots" on a plaster wall which has been painted without proper priming.

Brush application of the heretofore customary

primers has yielded fair results, but unless much time and effort is spent in working the primer over the surface, the primed surface is spotty and the spotty character persists after the surface is painted, injuring its appearance and decreasing 5 its resistance to weathering.

As a result of my investigations I have discovered a coating composition or "primer" for surfaces of zinc and other water-repellant metals, for example, galvanized metal which not only gives 10 excellent results when applied by spraying and entirely avoids the difficulties due to the spotty finish of prior primers, but also imparts to the surface a uniform and durable finish of any desired color and shade. This finish is not affected substantially 15 under the conditions to which ordinary roofing is exposed. Tests indicate that the finish given by the priming treatment of my invention will last for many years even when no coat of paint is placed over the primed surface. However, since 20 the priming treatment of my invention places the galvanized metal in excellent condition to receive and retain paint, I prefer, especially in the case of galvanized roofing, to use both paint and primer, employing a primer which imparts to the 25 roofing the same color as the subsequently applied paint, thus increasing the protection afforded to the roofing. Eventually the paint may come off the roofing in more exposed portions thereof, but inasmuch as the priming treatment 30 has imparted the same or nearly the same appearance to the underlying galvanized surface, repainting is necessary at infrequent intervals, if at all, and the roofing never acquires the leprous appearance often acquired by ordinary painted galvanized iron. 35

The primer of my invention comprises a mixture containing water, a water-soluble etching agent for water-repellant metal surfaces, a readily volatile, non-viscous, water-miscible organic liquid 40 which wets the surface more easily than does water and which does not react readily with the aqueous solution of the etching agent in the primer, and a pigment in the form of a water-insoluble compound of a heavy metal which does 45 not react readily with the aqueous solution of the etching agent in the primer.

I prefer to employ hydrochloric acid as the etching agent, but the other mineral acids, by which I mean sulphuric acid, nitric acid and 50 phosphoric acid, may also be used advantageously.

The readily volatile, water-miscible and non-viscous organic liquid in the primer acts as a "wetting" agent. I have found that acetone, methyl ethyl ketone, mono-ethyl ether of ethylene 55

glycol and the common lower alcohols such as methyl alcohol, ethyl alcohol and propyl alcohol are among the most satisfactory wetting agents to employ in the practice of my invention.

5 I prefer to use mineral pigments in the primer of my invention. By "mineral pigments" I mean finely divided, water-insoluble compounds of heavy metals (both natural and synthetic) such as the oxides of iron, chromium and titanium, barium sulphate, and complex pigments such as lithopone and titanated lithopone.

10 As indicated hereinbefore, the pigment employed should not be one which will be dissolved in large part by the aqueous solution of the etching agent in the primer under normal conditions of storage and use. Thus inert pigments such as barium sulphate are satisfactory, although I prefer to use pigments which are not substantially insoluble in the aqueous solution of the etching 15 agent in the primer. The oxides of iron, titanium and chromium (although not completely inert to the action of the mineral acids) are more satisfactory than inert pigments, because they become more firmly affixed to the treated surface. This I believe to be due to the fact that slight reaction between the etching agent and the pigment aids in fastening the latter to the treated surface. This may be due either to a 20 cementing action of the reaction products formed or it may be due to an alteration of the surface of the pigment particles which makes them adhere more firmly to zinc-base surfaces.

25 In addition to water, the etching agent, the wetting agent and the pigment, the primer of my invention preferably contains two other ingredients—a "deposition" agent and a "grease-cutting" agent.

30 By "deposition agent" I mean a water-soluble salt of a metal less electro-positive than zinc (or other water-repellant metal to be coated), such as copper sulphate, in which the metal, for example copper, tends to replace zinc and deposit on the zinc-base metal surface. The use of this 35 deposition agent is not essential but aids in obtaining a uniform surface for the application of paint.

35 Practically all galvanized iron and other fabricated forms of zinc coated metal have a thin non-uniform and usually invisible film of oil or grease upon them (at least in patches) which 40 has attached to the metal during fabrication or during subsequent handling. In order for the primer to act upon the metal surface it is necessary that it penetrate or remove this film of grease or oil. Otherwise the film will interfere 45 with uniform etching. The grease-cutting agent enables the primer to penetrate the film. The agent should be an organic solvent for hydrocarbons of the paraffin series. In addition it must be miscible with the wetting agent in the primer. Toluol, carbon tetrachloride and their homologues 50 are preferred examples of grease-cutting agents to be employed.

55 In practically all industrial applications it is safer to include the grease-cutting agent in the primer of my invention. If, however, it is certain that the metal surface to be treated has no grease or oil on it, the grease-cutting agent may be eliminated from the primer and replaced by an equal volume of wetting agent.

60 It is necessary that all of the ingredients employed in the primer be compatible with each other in the final mixture. Thus the wetting agent selected must be a solvent both for water and the grease-cutting agent. Otherwise, the

various liquids will separate out in layers, greatly impairing the effectiveness of the primer. Ethyl alcohol, for example, is soluble both in water and in carbon tetrachloride. It therefore acts not only as a wetting agent but also as a so-called 5 blending agent for the water and carbon tetrachloride which are not mutually soluble.

65 The action of the wetting agent in the practice of my invention is believed to be somewhat analogous to the action of a flotation agent in ore dressing. Mineral particles having metallic surfaces are water-repellant but are wetted by flotation agents. Consequently when a mixture of mineral particles some of which have non-metallic surfaces (quartz, feldspar) and others of 10 which have metallic surfaces (pyrite, galena) are 15 agitated vigorously in the presence of water and a flotation agent (pine oil), the flotation agent attaches to the particles having metallic surfaces and to air bubbles resulting from the agitation 20 and are thus buoyed up in a froth which is easily skimmed.

25 Metal surfaces of zinc, cadmium, magnesium and alloys of these metals of which zinc, cadmium or magnesium predominate have a "greasy" 25 quality even when they are absolutely clean. In other words, such surfaces are water-repellant. In consequence, when a strictly aqueous liquid is sprayed on such a surface it tends to collect thereon as minute drops and does not tend to 30 spread into a uniform film. This is especially true of galvanized sheets and the like where the coarsely crystalline character of the metal makes the surface irregular and bumpy; and thus introduces a further obstacle to the flow or spread of 35 the drops over the surface.

35 However, when a suitable wetting agent for the particular metal, say zinc, is included in the sprayed liquid the drops spread upon contact with the surface of the metal, eventually flow into each 40 other and produce a continuous liquid film through which the etching agent and the pigment particles may flow freely and thus become distributed on the surface with substantial uniformity. This results in an even distribution 45 and an intimate relationship between the etching agent in the aqueous solution and the pigment particles, with the result that the metal surface is etched uniformly.

50 I believe that the wetting agent in the primer, in addition to overcoming the difficulties described hereinbefore in a manner analogous to that of a flotation agent in ore dressing, also aids in dispersing the pigments in the primer. This is manifested by the tendency of the pigmented primer of my invention to become 55 "smooth" with much less stirring than is required with a suspension of pigments in a fluid which does not contain a wetting agent. The improved dispersion of pigments in the primer of my invention may be due to the more thorough wetting of the pigments by the fluids, but whatever be the explanation, the improved dispersion which is attained in the practice of my invention facilitates the uniform application of the primer 60 by spraying and precludes the presence of large agglomerates of pigment particles.

65 Apparently, during the etching process the pigment particles become affixed to the surface. I believe that the adhesion of the pigment particles to the metal surface without any conventional film forming ingredients to hold them 70 there is due to adsorption. In any case, the fact remains that the pigment particles become affixed to the surface even in the absence of any 75

of the customary film forming ingredients such as nitrocellulose or linseed oil.

My invention will be more completely understood if reference is made to the following detailed description of my present preferred practice.

*Preparation of the primer*

I first make up a clear primer which contains:

|    | Ingredient                                                                                   | Parts by volume |
|----|----------------------------------------------------------------------------------------------|-----------------|
| 15 | 30% copper sulphate solution (2½ lbs. CuSO <sub>4</sub> ·5H <sub>2</sub> O per gallon water) | 3½              |
| 15 | Commercial concentrated hydrochloric acid (containing about 35% by weight HCl)               | 5               |
|    | Carbon tetrachloride                                                                         | 5               |
|    | Toluol                                                                                       | 25              |
|    | "Cellosolve" mono-ethyl ether of ethylene glycol                                             | 10              |
| 20 | Denatured ethyl alcohol                                                                      | 5½              |
|    | Total                                                                                        | 100             |

The clear primer may be made up conveniently in 100 gallon batches in which case the parts by volume in the above formula may be taken as gallons. No special procedure is necessary in making up the clear primer. The ingredients are simply mixed together vigorously for a period of about 15 minutes, preferably in an acid-proof vessel.

The proportions of ingredients in the clear primer may be varied within moderately wide limits without impairing the final results. In general, however, the total volume of water, etching agent and deposition agent should range from 5 to 10% of the total. The wetting agents should comprise from 60 to 75% of the total volume, and the grease-cutting agents should be about 25 to 35% of the total volume. In this connection it should be noted that the mono-ethyl ether of ethylene glycol is one of the most desirable wetting agents to incorporate, to some extent at least, in the primer because it acts as a blending agent for the other liquid ingredients and permits a wider variation in the proportions of the other liquid ingredients in the primer.

To the clear primer is added the mineral pigments to give the desired color to the treated surface. The pigment should be acid-resistant and for optimum results it should be fine enough to pass completely through a screen having 325 meshes to the inch. In general, the mineral oxide pigments such as chrome green, red iron oxide, black iron oxide and titanium dioxide are to be preferred, but acid resistant sulphates such as barium sulphate and compound pigments such as lithopone and titanated lithopone may be employed advantageously. The following tabulation gives the preferred proportions of some pigments to clear primer:

|    | Color | Pigments                                   | Ounces of dry pigment per gallon of clear primer |
|----|-------|--------------------------------------------|--------------------------------------------------|
| 65 | Green | Chrome oxide                               | 10                                               |
|    | Red   | Red iron oxide                             | 8                                                |
| 70 | Black | Black iron oxide                           | 8                                                |
|    | Slate | (Black iron oxide 6<br>Titanium dioxide 2) | 8                                                |
|    | Brown | (Red iron oxide 6<br>Chrome oxide 3)       | 9                                                |

In mixing the clear primer and the pigment the latter is first worked into a paste with a small proportion of the primer. Working is continued until the paste is uniform and free of lumps, after which the balance of the primer is added and the whole is stirred together until the mixture is uniform and of a thin consistency.

*Coating the metal surfaces*

10

The pigmented primer may be applied by brushing or by dipping, but spray application is preferable. My invention, therefore, contemplates a process for producing a protective coating on the surface of zinc or similar water-repellent metal or alloy which comprises spraying the surface with a fluid mixture containing water, mineral acid, a mineral pigment and a volatile non-viscous and water-miscible organic liquid which does not react readily with the aqueous solution of the mineral acid in the mixture and which wets the surface more easily than does water, and permitting the surface to dry, whereby the surface becomes etched with substantial uniformity and the pigment adheres thereto.

During the spray application of the fluid mixture, the pigment should be kept in suspension. This is preferably accomplished by agitating the fluid mixture in the reservoir which fills the spray.

Preferably also, the grease-cutting agent or the deposition agent hereinbefore described are included in the fluid mixture which is sprayed.

In greater detail, the application of the pigmented primer to the water-repellent metal surface, for example, galvanized sheet iron shingles, should be conducted as follows:

Any visible grease or oil spots on the surface of the shingles is first removed by washing with an appropriate solvent such as naphtha.

The pigmented primer is charged into an acid proof container, such as a wooden keg, equipped with an agitator and acting as a reservoir for a pneumatic spray gun having an acid proof nozzle and needle. The pigmented primer in the reservoir should be agitated throughout the period of spray application.

The clean shingle surface is then sprayed as uniformly as possible. The spray should be fine and evenly distributed in a fan shape. With the customary paint spray gun the air pressure when the spray is open should be approximately 40 pounds, and the valve which supplies the pigmented primer to the spray should be opened only slightly; otherwise an excessive spray results. The sprayed coat of primer while wet should show definitely the pattern of the spangles on the surface of the galvanized shingles. If the pattern of the spangles is obscured, too much primer has been used.

After the primer is sprayed on the shingles, they should be stacked carefully in a dry atmosphere and permitted to dry for at least 5 hours and preferably overnight. On rainy days or when the humidity is exceptionally high this drying period should be prolonged up to a maximum of about 24 hours.

One spray coat of primer is sufficient, but in no case should paint be applied over the primer surface until it is completely dry. One gallon of the primer will cover 450 to 500 square feet of surface if the primer is properly applied.

The containers, spray pots, spray guns and

hose which are used for applying the primer should not be used for any other purpose, such as for spraying paint. Admixture of the primer with paint spoils the paint and vice versa.

5 When changing from one color of primer to another, the interior of the entire spray apparatus should be cleaned with water.

As hereinbefore indicated, it is not necessary to apply paint over the primed surface because 10 the primer itself imparts to the roofing a durable coating of any desired color or shade. However, the primed surface furnishes an excellent base for paint, particularly for the paint described hereinafter and presents an outstanding advantage 15 over primers proposed heretofore in that paint can be applied directly over the dry primer coat, without first washing the primed surface or otherwise treating it to remove reaction products. Consequently, to give additional protection for 20 the surface I prefer to apply at least one spray coat of paint over the primed surface, using paint of the same color as the pigmented primer. The paint gradually "chalks" from the surface during exposure to the weather, but even after the paint 25 is entirely gone the roof will still give many years of service and will appear unaltered in color both during the time when the paint is chalking off and thereafter.

Almost any paint may be used to cover the 30 primed shingle surface. However, I have discovered that it is best to employ paint which "chalks" when exposed to the weather, i. e. paint which fails gradually and washes off the painted surface as an impalpable powder or mud during 35 long periods of exposure. A paint of this character is desirable because it does not fail in patches and therefore gives additional security that the roof will not acquire a spotty appearance due to the fact that on some portions of it paint 40 still remains while on other portions the paint has been removed, exposing a primed surface which is of slightly different appearance.

I have developed an especially suitable paint 45 which comprises a varnish base made by cooking China-wood oil with a phenol formaldehyde resin together with a high proportion of "filler" such as talc or barytes. This paint is especially applicable in the practice of my invention not only because 50 it does not fail in patches but also because it adheres well to the primed surface and give an unusually uniform finish.

The varnish is prepared by cooking about 4 parts by weight of phenol formaldehyde resin with 55 about 16 parts by weight of China-wood oil for about half an hour at a temperature not to exceed 480° F. The mixture thus formed is allowed to cool and 26 parts by weight of mineral spirits is mixed with it thereafter. About 1 part 60 by weight of dryer (for example a mixture of powdered cobalt, manganese and lead in the proportion 4-16-80 by weight) is then added to the varnish.

The pigment employed in the paint should be 65 the same in fineness and color as the pigment in the primer. However, the chemical composition of the pigment in the paint need not be the same as that in the primer because the pigment in the paint need not be acid resistant to the same degree. Thus, when green shingles are desired, chrome green should be used as the pigment in the primer, but a mixture of Prussian blue and lead chromate which will give the same shade and 70 color of green may be used in the paint.

A preferred formula for the paint to apply over the primed surface is as follows:

| Ingredients                                                                           | Amounts   | 5  |
|---------------------------------------------------------------------------------------|-----------|----|
| Hiding pigment (dry colors such as a mixture of Prussian blue and lead chromate)..... | 200 lbs.  |    |
| Talc.....                                                                             | 200 lbs.  |    |
| Barytes.....                                                                          | 800 lbs.  |    |
| Varnish vehicle prepared as hereinbefore described.....                               | 100 gals. |    |
| Additional thinner—turpentine substitute or naphtha.....                              | 44 gals.  | 10 |

A portion of the varnish is used as a grinding medium for the pigment and filler. Grinding may be carried out conveniently in a pebble mill or the like. A stiff paste is thus formed. Thereafter the balance of the liquid ingredients of the paint is added.

The above produces approximately 178 gallons of heavy paint. Before use this should be thinned with one part of naphtha or mineral thinner for each three parts of the paint.

The thinned paint should be applied over the dry primed surface with an ordinary pneumatic spray gun, using sufficient paint to cover the surface adequately. It has been found that one gallon of the paint described hereinbefore will adequately cover about 400 square feet. Only one coat of this paint is necessary.

Good results have been obtained with an air pressure of from 30 to 40 pounds per square inch when the gun is open and with the paint valve on the gun open but slightly so as to produce a fine spray.

After painting, the finished articles should be dried for at least 24 hours before they are packed for shipment. The paint described above acquires a flat and dry appearance within a few minutes after it is applied, but it does not harden to the extent required for handling until it has dried at room temperature for at least 12 hours.

Care should be taken to assure that the primed surface is absolutely dry before paint is applied over it and also to assure that the paint does not come in contact with the wet primer at any time. This means that the containers, hose, spray gun and any other apparatus with which the paint comes in contact should not be used for handling the primer.

I claim:

1. A process for producing a protective coating on a water-repellant metal surface selected from the group consisting of zinc, cadmium, magnesium and alloys of these metals which comprises spraying said surface with a fluid mixture containing water, mineral acid, a volatile, non-viscous and water-miscible organic liquid which does not react readily with the aqueous solution of the mineral acid in the mixture and which readily wets the surface and more easily than does water, and a substantially water-insoluble mineral pigment which is resistant to the acid in the mixture, and permitting said surface to dry, whereby a reaction occurs which etches the surface with substantial uniformity and causes the pigment to adhere thereto.

2. A process for producing a protective coating on a water-repellant surface of metal selected from the group consisting of zinc, cadmium and magnesium and alloys in which one or more of these metals constitute a major ingredient which comprises spraying said surface with a fluid mixture containing water, a mineral acid, a volatile non-viscous and water-miscible organic liquid which does not react readily with the mineral acid in the mixture and readily wets said surface and

- more readily than does water and a pigment in the form of a water-insoluble oxide of a heavy metal, said pigment being resistant to the acid in said mixture, permitting the resulting primed 5 surface to dry, whereby a reaction occurs which causes the surface to become etched and the pigment to adhere to the etched surface and while retaining on the dry surface a reaction product of the metal and the mineral acid spraying the 10 dry surface with a paint of substantially the same color as the pigment and which fails by chalking upon continued exposure to the weather.
3. A process for producing a protective coating on a greasy galvanized metal surface which comprises spraying the surface with a fluid primer containing water, a mineral acid, a wetting agent in the form of a volatile non-viscous and water-miscible organic liquid which readily wets zinc and more easily than does water and does not 15 react readily with the mineral acid in the mixture at room temperature, an organic solvent for the grease on the galvanized metal surface which is miscible with the wetting agent and a pigment in the form of a water-insoluble oxide of a heavy 20 metal which is resistant to the acid in the primer, and drying the sprayed surface whereby a reaction occurs which causes the surface to become etched with substantial uniformity and the pigment to adhere to the etched surface.
- 30 4. A process for producing a protective coating on a water-repellant surface of metal selected from the group consisting of zinc, cadmium, magnesium and alloys containing one or more of these metals as a major ingredient which comprises incorporating a substantially water-insoluble acid-resistant mineral pigment into a fluid mixture containing water, mineral acid, a volatile non-viscous and water-miscible organic liquid which does not react readily with the aqueous solution of the mineral acid in the mixture and which readily wets the surface and more easily than does water, spraying the resulting 35 pigmented mixture on said surface while maintaining the pigment in suspension in the mixture, the coating of primer being applied to the surface in such quantity that while the surface is still wet the spangles are apparent, and permitting said surface to dry, whereby the surface becomes etched and the pigment adheres to the etched 40 surface.
5. Process according to claim 4 in which the pigment mixture is agitated in a reservoir before being sprayed and the agitation is continued substantially throughout the time of spraying.
6. A process for producing a protective coating on water-repellant surfaces of metals and alloys containing a metal selected from the group consisting of zinc, cadmium and magnesium which comprises incorporating a mineral pigment selected from the group consisting of iron, chromium and titanium oxides, barium sulphate and lithopone into a fluid mixture containing water, mineral acid, a volatile non-viscous and water-miscible organic liquid which does not react readily with the aqueous solution of the mineral acid in the mixture and which readily wets the surface and more easily than does water, the proportions of pigment to liquid in the mixture being about 10 ounces per gallon, spraying the resulting pigmented mixture on said surface while maintaining the pigment in suspension in the mixture, and permitting said surface to dry whereby the surface becomes etched with substantial uniformity and the pigment in the mixture adheres to the etched surface.
7. A process for producing a protective coating on a spangled galvanized surface which comprises incorporating a mineral pigment selected from the group consisting of iron, chromium and titanium oxides, lithopone and barium sulphate into a fluid mixture containing water, mineral acid, a volatile non-viscous and water-miscible organic liquid which does not react readily with the aqueous solution of the mineral acid in the mixture and which readily wets the surface and more easily than does water, spraying the resulting pigmented mixture on the surface while maintaining the pigment in suspension in the mixture, the coating of primer being applied to the surface in such quantity that while the surface is still wet the spangles are apparent, and permitting said surface to dry, whereby the surface becomes etched and the pigment adheres to the etched surface.

WILLIAM E. HALL.